# EUROPEAN PATENT SPECIFICATION

(11) **EP 0 654 148 B1**
(45) Date of publication and mention of the grant of the patent: **15.10.1997**
(21) Application number: 93916592.4
(22) Date of filing: 22.06.1993
(51) Int. Cl.: G03C 5/30, G03C 5/305

(54) **USE OF KETOGLUCONATES IN PHOTOGRAPHY**
VERWENDUNG VON KETOGLUCONATEN IN DER PHOTOGRAPHIE
UTILISATION DE CETOGLUCONATES EN PHOTOGRAPHIE

(30) Priority: 05.08.1992 US 926092
(43) Date of publication of application: 24.05.1995
(73) Proprietor: Cultor Ltd., 00240 Helsinki (FI)
(72) Inventor: GEWANTER, Herman L., Waterford, CT 06385 (US); RASHAN, Joseph M., Jr., Waterford, CT 06385 (US); REITZ, Larry R., Salem, CT 06420 (US)
(74) Representative: Patentanwälte Zellentin & Partner
(86) International application number: US9305802
(87) International publication number: WO9403834

(56) References cited:
- EP-A- 0 508 691
- GB-A- 1 467 007
- US-A- 4 551 411
- DATABASE WPI Week 8841, Derwent Publications Ltd., London, GB; AN 88-290784 (41) & SU,A,1 381 416 (LENGD CINE ENGR INS) 15 March 1988
- DATABASE WPI Week 8841, Derwent Publications Ltd., London, GB; AN 88-290784 (41)

## Description

The present invention relates to the use of derivatives of ketogluconic acid as photographic agents.

Development of a photographic image (both negative and positive) is accomplished by selective reduction of light sensitized silver halide to elemental silver. Chemicals capable of this selective reduction are generally of the "Kendall Structure"

X₁-(C=C)ₙ-X₂

wherein X₁ and X₂ are hydroxy, amino or substituted amino group and n is either zero or an integer.

Silver halide emulsions are coated on various papers and films for use in photographic applications. When these emulsions have been exposed to radiation, the sensitized emulsion produces a latent image in the silver halide grains. The image is latent because the grains are sensitized to reduction by the formation of minute quantities of free silver in the grains from the exposure. These grains are developed by placing the exposed photosensitive material in an aqueous solution containing one or more specific reducing chemicals. There are very few reducing agents which will only develop the latent image and not reduce the unexposed silver halide. The reducing agents conventionally employed include such organic materials as hydroquinone and other materials meeting the criteria of the Kendall-Pelz rule.

The structure of developing agents according to the rule are as follows:

a-(A=B)-a'

where
A is carbon,
B is carbon or nitrogen,
a and a' are OH, NH₂, NHR₁, NR₁R₂.
Examples of chemicals meeting this rule are hydroquinone, catechol, pyrogallol, ascorbic acid and its stereoisomers, and derivatives of phenylenediamine. An example of a developing agent which is an exception to the rule is 1-phenyl-3-pyrazolidone (Phenidone).

Two of these developing agents may be used in the same formulation to produce a result known in the photographic industry as superadditivity, also known as synergy. It is defined as the mixture of two developing agents showing a greater degree of developer activity than the sum of the actions of each agent separately.

Figs. 1-6 are graphs showing the effect of various ketogluconates on photographic media.

In one embodiment, the present invention is directed to a process for the development of a photographic image on a photographic medium comprising reducing the photosensitized silver on said medium with an effective amount of (a) a compound selected from the group consisting of alkali metal salts, alkaline earth metal salts, amine salts of ketogluconic acid, alkali metal salts, alkaline earth metal salts and amine salts of stereoisomers of ketogluconic acid; and C₁-C₄ alkyl esters of ketogluconic acid and C₁-C₄ alkyl esters of stereoisomers of ketogluconic acid; and (b) a co-developer.

In a preferred process, the salt of ketogluconic acid is sodium-2-ketogluconate.

In an especially preferred process, the ester is the methyl ester.

In another preferred process, the methyl ester is methyl-2-ketogluconate.

In another especially preferred process, the alkaline earth metal salt is calcium-2,5-diketogluconate.

In a preferred process, the co-developer is selected from the group consisting of 4-methylaminophenol, 1-phenyl-3-pyrazolidone, and para-phenylenediamines.

In a further embodiment, the present invention is directed to a photographic composition comprising (a) an effective amount of a developing agent selected from the group consisting of alkali metal salts, alkaline earth metal salts, amine salts of ketogluconic acid; alkali metal salts, alkaline earth metal salts and amine salts of stereoisomers thereof; C₁-C₄ alkyl esters of said salts of ketogluconic acid and stereoisomers thereof; and (b) a co-developer.

In a preferred composition the co-developer is selected from the group consisting of 4-methylaminophenol, 1-phenyl-3-pyrazolidone, and para-phenylenediamines.

In another embodiment, the present invention is directed to a process for the development of a photographic image on a photographic medium comprising reducing the photosensitized silver on said medium with an effective amount of methyl-2-ketogluconate.

In another embodiment, the present invention is directed to a photographic composition containing an effective amount of methyl-2-ketogluconate as a developing agent.

The present invention uses derivatives of ketogluconic acid. These derivatives are used in the form of salts which are hereinafter referred to as either ketogluconates or in the case of the stereoisomers, as ketogulonates.

One class of the present developing agents are the alkali metal salts of keto-gluconates, and stereoisomers thereof. The D, L and DL forms of the keto-gluconates may be used. Stereoisomers of the ketogluconates include the ketogulonates which may also be used in the D, L or DL forms.

Preferred alkali metal salts are the sodium and potassium salts. The sodium and potassium salts of the keto-D-gluconates, keto-L-gluconates, and the keto-DL-gluconates may be used in the composition and process of the present invention. Similarly, the sodium and potassium salts of the keto-D-gulonates, keto-L-gulonates and keto-DL-gulonates may be used in the process and compositions of the present invention.

Preferred amine salts are the ammonium salts, the triethanolamine salts, the diethylaminoethyl, cyclohexylamine, and the morpholine salts of the ketogluconates and ketogulonates.

Preferred alkaline earth metal salts are the calcium salts of ketogluconates and ketogulonates.

As is well known to these skilled in the art to which this invention applies, the derivatives of ketogluconic acid also exist in the diketo form. Thus, as used herein, salts of ketogluconic acid include the diketo salts and esters include the diketo esters.

Preferred esters of the ketogluconates and ketogulonates are the C₁-C₄ alkyl esters. Preferred is the methyl ester.

The derivatives of ketogluconic acid are used with a co-developer. Preferred co-developers are metol (1-phenyl-3 pyrazolidone), a pyrazolidone derivative, phenidone (4-aminomethylphenol), and para-phenylenediamines.

Other 3-pyrazolidone silver halide developing agents may be used. Examples of such derivatives include: 1-p-tolyl-3-pyrazolidone, 5-phenyl-3-pyrazolidone, 5-met-3-pyrazolidone, 1-p-chlorophenol-3-pyrazolidone, 1-phenyl-5-phenyl-3-pyrazolidone, m-tolyl-3-pyrazolidone, 1-phenyl-5-methyl-3-pyrazolidone, 1-p-tolyl-5-phenyl-3-pyrazolidone, 1-m-tolyl-3-pyrazolidone, 1-p-methoxyphenyl-3-pyrazolidone, 1-acetamidophenyl-3-pyrazolidone, 1-phenyl-2-acetyl-4, 4-dimethyl-3-pyrazolidone, 1-phenyl-4, 4-dimethyl-3-pyrazolidone, 1-m-aminophenyl-4-4-propyl-3-pyrazolidone, 1-o-chlorophenol--4.methyl-4-ethyl-3-pyrazolidone, 1-m-acetarnidophenyl-4, 4-diethyl-3-pyrazolidone, 1-p-hydroxyphenyl-4, 4-dimethyl-3-pyrazolidone, 1-p-methoxyphenyl-4, 4-diethyl-3-pyrazolidone, 1-p-tolyl-4,4-dimethyl-3-pyrazolidone, 1-p-diphenyl-4,4-dimethyl3-pyrazolidone,1-p-(B-hydroxyethylphenyl)-3-pyrazolidone,1-o-tolyl-3-pyrazolidone,1-o-tolyl-4,4-dimethyl-3-pyrazolidone.

Examples of phenylenediamine compounds are N,N-diethyl-p-phenylene-diamine, N,N-diethyl-o-methyl-p-phenylenediamine, N,N-diethyl-methoxy-p-phenylenediamine, P-phenylenediamine, N-ethyl-n-hydroxyethyl-p-phenylenediamine, and N-ethyl-N-hydroxyethyl-o-methyl-p-phenylenediamine.

Examples of photographic media on which images may be developed include black and white print film, color transparencies, black and white transparencies, and color print film.

It has also been found that the methyl ester of ketogluconic acid, methyl-2-ketogluconate will develop an image without the presence of a co-developer. Thus, the present invention is also directed to a process for developing a photographic image by using methyl-2-ketogluconate as a developer, and to a photographic composition containing methyl-2-ketogluconate as a developing agent.

Having described the invention in general terms, reference is now made to specific examples. It is to be understood that these examples are not meant to limit the present invention, the scope of which is determined by the appended claims.

The developing formulations used in these procedures are based on universal developer solutions described in the S.P.S.E. Handbook of Photographic Science and Engineering, Wiley, 1973, page 569. Various derivatives of ketogluconic acid were substituted for those described in the formulations.

In the test to evaluate the developers on paper, a piece of commercial black and white photographic paper was exposed to a light source from an enlarger at a f-stop of 11 for 30 seconds. A 21 step wedge of various densities was in contact with the paper during exposure. The entire procedure was conducted under safelight conditions. After exposure the paper was developed in the test formulation for 2 minutes. The paper was then placed in an acid stop bath for 10 seconds. Following the stop, the paper was fixed in a Kodak F-5 formulation. The entire development procedure took place in trays placed in a temperature control shaker bath at a constant speed and 20 degree C. The paper was then rinsed in running water for 5 minutes and dried. The densities of the step wedge developed on the paper were then read on a Macbeth TR 924 densitometer. The results of the test were plotted on a D log E curve. The y axis had the values of densities from the relative step exposure on the x axis.

In order to evaluate our developers on film, the exposure and developing of the film took place in total darkness. The film was exposed in a X-Rite 383 sensitometer which has a built in 21 step wedge template. The film was then developed in a test formulation for 4 minutes, stopped for 10 seconds, and fixed (Kodak F-5) for 4 minutes. Again the entire development procedure took place at a constant agitation and a temperature of 20 degree C. The film was then washed in running water for 20 minutes, squeeged, and dried, and a D log E curve was prepared.

### Example 1

The following formulations were prepared and used to develop Kodak Polycontrast III RC FM paper.

| gram to 500 ml water | | | |
|---|---|---|---|
| sodium sulfite | 12.5 | 12.5 | 12.5 |
| | | | |
| hydroquinone | 3.0 | | |
| | | | |
| methyl-2-ketogluconate | | | 10.0 |
| | | | |
| sodium carbonate | 15.0 | 15.0 | 15.0 |
| | | | |
| phenidone | | 0.125 | |
| | | | |
| potassium bromide | 0.5 | 0.5 | 0.5 |
| | | | |
| benzotriazole | 0.05 | 0.5 | 0.05 |
| | | | |
| potassium hydroxide | | | 3.6 |

| Results of Development | | | |
|---|---|---|---|
| Relative Log Exposure Steps | Hydroquinone Formulation | Phenidone Formulation Densities | Methyl-2-ketogluconate Formulation Densities |
| 1 | 0.03 | 0.03 | 0.04 |
| 2 | 0.03 | 0.03 | 0.04 |
| 3 | 0.04 | 0.04 | 0.05 |
| 4 | 0.12 | 0.17 | 0.15 |
| 5 | 0.42 | 0.49 | 0.45 |
| 6 | 0.77 | 0.88 | 0.80 |
| 7 | 1.15 | 1.29 | 1.18 |
| 8 | 1.52 | 1.65 | 1.57 |
| 9 | 1.94 | 1.96 | 1.99 |
| 10 | 2.05 | 2.03 | 2.07 |
| 11 | 2.07 | 2.04 | 2.08 |

The results of this test indicate that methyl-2-ketogluconate is a developing agent and yields equivalent densities to those of hydroquinone and phenidone. The graph of this example is shown as Fig. 1.

### Example 2

The following formulations were prepared and used to develop Kodak Tri-X Pan 4164 film.

| gram to 500 ml water | | | |
|---|---|---|---|
| metol | 0.5 | | 0.5 |
| | | | |
| sodium sulfite | 12.5 | 12.5 | 12.5 |
| | | | |
| methyl-2-ketogluconate | | 12.0 | 12.0 |
| | | | |
| sodium carbonate | 18.0 | 18.0 | 18.0 |
| | | | |
| potassium bromide | 0.1875 | 0.1875 | 0.1875 |

| Results of Development | | | |
|---|---|---|---|
| Relative Log Exposure Steps | Metol Formulation Densities | Methyl-2-ketogluconate Formulation Densities | Metol/methyl-2 ketogluconate Formulation Densities |
| 1 | | 0.06 | 0.18 |
| 2 | 0.18 | 0.06 | 0.20 |
| 3 | 0.23 | 0.06 | 0.24 |
| 4 | 0.25 | 0.06 | 0.30 |
| 5 | 0.31 | 0.06 | 0.40 |
| 6 | 0.33 | 0.06 | 0.48 |
| 7 | 0.33 | 0.06 | 0.57 |
| 8 | 0.35 | 0.06 | 0.65 |
| 9 | 0.40 | 0.06 | 0.74 |
| 10 | 0.43 | 0.06 | 0.82 |
| 11 | 0.46 | 0.06 | 0.94 |
| 12 | 0.50 | 0.06 | 1.06 |
| 13 | 0.53 | 0.06 | 1.20 |
| 14 | 0.57 | 0.06 | 1.34 |
| 15 | 0.61 | 0.06 | 1.45 |
| 16 | 0.66 | 0.06 | 1.60 |
| 17 | 0.70 | 0.06 | 1.72 |
| 18 | 0.74 | 0.06 | 1.80 |
| 19 | 0.80 | 0.06 | 1.93 |
| 20 | 0.87 | 0.06 | 2.06 |
| 21 | 0.93 | 0.06 | 2.25 |

The results of this test show that methyl-2-ketogluconate has superadditivity with metol, since the sum of the active of the two compounds is greater than either one alone. The graph of the example is shown as Fig. 2.

### Example 3

The following formulations were prepared and used to develop Kodak Tri-X Pan 4164 film.

| gram to 500 ml water | | | |
|---|---|---|---|
| sodium sulfite | 12.5 | 12.5 | 12.5 |
| | | | |
| methyl-2-ketogluconate | | 12.0 | 12.0 |
| | | | |
| sodium carbonate | 15.0 | 15.0 | 15.0 |
| | | | |
| phenidone | 0.125 | | 0.125 |
| | | | |
| potassium bromide | 0.5 | 0.5 | 0.5 |
| | | | |
| benzotriazole | 0.05 | 0.5 | 0.05 |

The table above shows that methyl-2-ketogluconate is a co-developer with phenidone and displays superadditivity. Phenidone is preferred because it is commercially available in large quantities while other known, related developing agents having similar structures and characteristics are not widely available. The graph of the data is shown as Fig. 3.

### Example 4

The following formulations were prepared and used to develop Kodak Tri-X Pan 4164 film. The formula for N,N-Diethyl-1, 4-phenylenediamine will be abbreviated as DEPDA.

| gram to 500 ml water | | | |
|---|---|---|---|
| DEPDA | 0.241 ml | | 0.241 ml |
| | | | |
| sodium sulfite | 12.5 | 12.5 | 12.5 |
| | | | |
| methyl-2-ketogluconate | | 12.0 | 12.0 |
| | | | |
| sodium carbonate | 18.0 | 18.0 | 20.0 |
| | | | |
| potassium bromide | 0.1875 | 0.1875 | 0.1875 |

| Results of Development | | | |
|---|---|---|---|
| Relative Log Exposure Steps | DEPDA Formulation Densities | Methyl-2-ketogluconate Formulation Densities | DEPDA/Methyl-2-ketogluconate Formulation Densities |
| 1 | 0.12 | 0.06 | 0.18 |
| 2 | 0.12 | 0.06 | 0.20 |
| 3 | 0.12 | 0.06 | 0.22 |
| 4 | 0.14 | 0.06 | 0.24 |
| 5 | 0.16 | 0.06 | 0.30 |
| 6 | 0.18 | 0.06 | 0.34 |
| 7 | 0.19 | 0.06 | 0.40 |
| 8 | 0.21 | 0.06 | 0.45 |
| 9 | 0.23 | 0.06 | 0.51 |
| 10 | 0.25 | 0.06 | 0.57 |
| 11 | 0.27 | 0.06 | 0.64 |
| 12 | 0.30 | 0.06 | 0.71 |
| 13 | 0.32 | 0.06 | 0.79 |
| 14 | 0.36 | 0.06 | 0.90 |
| 15 | 0.38 | 0.06 | 0.99 |
| 16 | 0.40 | 0.06 | 1.09 |
| 17 | 0.42 | 0.06 | 1.21 |
| 18 | 0.48 | 0.06 | 1.36 |
| 19 | 0.51 | 0.06 | 1.51 |
| 20 | 0.50 | 0.06 | 1.66 |
| 21 | 0.57 | 0.06 | 1.85 |

These results demonstrate superadditivity of methyl-2-ketogluconate with another developing agent. The graph is shown as Fig. 4.

### Example 5

The following formulation was prepared and used to develop Kodak Polycontrast III RC FM paper.

| grams to 500 ml with water | | Relative Log Exposure Steps | Densities |
|---|---|---|---|
| sodium sulfite | 12.5 | 1 | 0.15 |
| calcium-2,5- | 6.0 | 2 | 0.21 |
| diketogluconate | | 3 | 0.21 |
| sodium carbonate | 15.0 | 4 | 0.20 |
| potassium bromide | 0.5 | 5 | 0.57 |
| benzotriazole | 0.05 | 6 | 0.90 |
| pH to 11.3 with KOH | | 7 | 1.26 |
| | | 8 | 1.66 |
| | | 9 | 2.00 |
| | | 10 | 2.07 |
| | | 11 | 2.08 |

This data indicates that other ketogluconates can have activity as photographic developers. The graph is shown as Fig. 5.

### Example 6

The following formulation was prepared and used to develop Kodak KODAUTH Ortho film, Type 3.

| gram to 500 ml with water | | Relative Log Exposure Steps | Densities |
|---|---|---|---|
| sodium sulfite | 12.5 | 1 | 0.24 |
| methyl-2- | | 2 | 0.24 |
| diketogluconate | 40.0 | 3 | 0.24 |
| sodium | | 4 | 0.24 |
| carbonate | 18.0 | 5 | 0.24 |
| potassium | | 6 | 0.24 |
| bromide | 0.1875 | 7 | 0.24 |
| pH 10.5 with KOH | | 8 | 0.25 |
| | | 9 | 0.25 |
| | | 10 | 0.25 |
| | | 11 | 0.25 |
| | | 12 | 0.25 |
| | | 13 | 0.25 |
| | | 14 | 0.26 |
| | | 15 | 0.26 |
| | | 16 | 0.26 |
| | | 17 | 0.27 |
| | | 18 | 0.31 |
| | | 19 | 0.39 |
| | | 20 | 0.63 |
| | | 21 | 1.54 |

This data shows that methyl-2-ketogluconate will produce an image on film without co-developers. The graph is shown as Fig. 6.

## Claims (Claims for the following Contracting State(s): AT, CH, DK, ES, GR, IE, LI, LU, PT, SE)

1. A process for the development of a photographic image on a photographic medium comprising reducing the photosensitized silver on said medium with an effective amount of (a) a compound selected from the group consisting of alkali metal salts, alkaline earth metal salts, and, amine salts of ketogluconic acid; alkali metal salts, alkaline earth metal salts, and, amine salts of stereoisomers of ketogluconic acid, and C₁-C₄ alkyl esters of ketogluconic acid, C₁-C₄ alkyl esters of stereoisomers of ketogluconic adid, and (b) a co-developer for said photographic medium.

2. A process according to claim 1 wherein said salt of keto-gluconic acid is sodium 2-ketogluconate.

3. A process according to claim 1 wherein said ester is the methyl ester.

4. A process according to claim 3 wherein said methyl ester is methyl 2-ketogluconate.

5. A process according to claim 1 wherein said alkaline earth metal salt is calcium-2,5-diketogluconate.

6. A process according to claim 1 wherein said co-developer is selected from the group consisting of methylaminophenol, 1-phenyl-3-pyrazolidone and para-phenylenediamines.

7. A photographic material containing an effective amount of a developing agent selected from the group consisting of alkali metal salts, alkaline earth metal salts, amine salts of ketogluconic acid; alkali metal salts, alkaline earth metal salts and amine salts of stereoisomers thereof; C₁-C₄ alkyl esters of ketogluconic acid, and C₁-C₄ alkyl esters of stereoisomers of ketogluconic acids, and (b) a co-developer in said photographic medium.

8. A material according to claim 7 where said co-developer is selected from the group consisting of methylaminophenol, 1-phenyl-3-pyrazolidone and para-phenylenediamines.

9. A process for the development of a photographic image on a photographic medium comprising reducing the photosensitized silver on said medium with an effective amount of methyl-2-ketogluconate.

10. A photographic material containing an effective amount of methyl-2-ketogluconate as a developing agent.

## Claims (Claims for the following Contracting State(s): BE, DE, FR, GB, IT, NL)

1. A process for the development of a photographic image on a photographic medium comprising reducing the photosensitised silver on said medium with an effective amount of (a) calcium-2,5-diketogluconate and (b) a co-developer for said photographic medium.

2. A process according to claim 1 wherein said co-developer is selected from the group consisting of methylaminophenol, 1-phenyl-3-pyrazolidone and paraphenylenediamines.

3. A photographic material containing an effective amount of calcium-2,5-diketogluconate and a co-developer in said photographic medium.

4. A photographic material according to claim 3 where said co-developer is selected from the group consisting of methylaminophenol, 1-phenyl-3-pyrazolidone and paraphenylenediamines.

## Patentansprüche (Patentansprüche für folgende(n) Vertragsstaat(en): AT, CH, DK, ES, GR, IE, LI, LU, PT, SE)

1. Verfahren zur Entwicklung von fotografischen Bildern auf einem fotografischen Medium, welches darin besteht, fotosensibilisiertes Silber auf besagtem Medium zu reduzieren, mit einer ausreichenden Menge von (a) einer Substanz ausgewählt aus der Gruppe bestehend aus Alkalimetallsalzen, Erdalkalimetallsalzen und Aminsalzen von Ketogluconsäure; Alkalimetallsalzen, Erdalkalimetallsalzen und Aminsalzen von Stereoisomeren von Ketogluconsäure und C₁-C₄-Alkylestern von Ketogluconsäure, C₁-C₄-Alkylestern von Stereoisomeren von Ketogluconsäure und (b) einem Co-Entwickler für das fotografische Medium.

2. Verfahren gemäß Anspruch 1, **dadurch gekennzeichnet**, daß das Salz der Ketogluconsäure ein Natrium-2-ketogluconat ist.

3. Verfahren gemäß Anspruch 1, **dadurch gekennzeichnet,** daß der Ester ein Methylester ist.

4. Verfahren gemäß Anspruch 3, **dadurch gekennzeichnet**, daß der Methylester ein Methyl-2-ketogluconat ist.

5. Verfahren gemäß Anspruch 1, **dadurch gekennzeichnet,** daß das Erdalkalimetallsalz Calcium-2,5-diketogluconat ist.

6. Verfahren gemäß Anspruch 1, **dadurch gekennzeichnet**, daß der Co-Entwickler ausgewählt ist aus der Gruppe bestehend aus Methylaminophenol, 1-Phenyl-3-pyrazolidon und Paraphenylendiaminen.

7. Fotografisches Material, welches eine ausreichende Menge eines Entwicklungsmittels ausgewählt aus der Gruppe bestehend aus Alkalimetallsalzen, Erdalkalimetallsalzen, Aminsalzen von Ketogluconsäure; Alkalimetallsalzen, Erdalkalimetallsalzen und Aminsalzen von Stereoisomeren davon; C₁-C₄-Alkylestern von Ketogluconsäure und C₁-C₄-Alkylestern von Stereoisomeren von Ketogluconsäuren und (b) ein Co-Entwickler in dem fotografischen Medium besteht.

8. Material gemäß Anspruch 7, **dadurch gekennzeichnet**, daß der Co-Entwickler ausgewählt ist aus der Gruppe bestehend aus Methylaminophenol, 1-Phenyl-3-pyrazolidon und Paraphenylendiaminen.

9. Verfahren für die Entwicklung eines fotografischen Bildes auf einem fotografischen Medium bestehend aus der Reduktion des fotosensibilisierten Silbers auf besagtem Medium mit einer ausreichenden Menge von Methyl-2-ketogluconat.

10. Fotografisches Material enthaltend eine ausreichende Menge von Methyl-2-ketogluconat als Entwicklungsmittel.

## Patentansprüche (Patentansprüche für folgende(n) Vertragsstaat(en): BE, DE, FR, GB, IT, NL)

1. Verfahren zur Entwicklung von fotografischen Bildern auf einem fotografischen Medium, bestehend aus der Reduktion des fotosensibilisierten Silbers auf besagtem Medium mit einer ausreichenden Menge von (a) Calcium-2,5-diketogluconat und (b) einem Co-Entwickler für das fotografische Medium.

2. Verfahren gemäß Anspruch 1, **dadurch gekennzeichnet,** daß der Co-Entwickler ausgewählt ist aus der Gruppe bestehend aus Methylaminophenol, 1-Phenyl-3-pyrazolidon und Paraphenylendiamin.

3. Fotografisches Material enthaltend eine ausreichende Menge von Calcium-2,5-diketogluconat und einen Co-Entwickler in dem fotografischen Medium.

4. Fotografisches Material gemäß Anspruch 3, **dadurch gekennzeichnet,** daß der Co-Entwickler ausgewählt ist aus der Gruppe bestehend aus Methylaminophenol, 1-Phenyl-3-pyrazolidon und Paraphenylendiaminen.

## Revendications (Revendications pour l'(les) Etat(s) contractant(s) suivant(s): AT, CH, DK, ES, GR, IE, LI, LU, PT, SE)

1. Procédé pour le développement d'une image photographique sur un support photographique comprenant la réduction de l'argent photosensibilisé sur ledit support avec une quantité efficace de (a) un composé choisi dans le groupe constitué des sels de métaux alcalins, sels de métaux alcalino-terreux, et, sels d'amine de l'acide cétogluconique; des sels de métaux alcalins, sels de métaux alcalino-terreux, et, sels d'amine des stéréoisomères de l'acide cétogluconique, et des esters alkyliques en C₁-C₄ de l'acide cétogluconique, des esters alkyliques en C₁-C₄ des stéréoisomères de l'acide cétogluconique, et de (b) un co-révélateur pour ledit support photographique.

2. Procédé selon la revendication 1, dans lequel ledit sel de l'acide cétogluconique est le 2-cétogluconate de sodium.

3. Procédé selon la revendication 1, dans lequel ledit ester est l'ester méthylique.

4. Procédé selon la revendication 3, dans lequel ledit ester méthylique est le 2-cétogluconate de méthyle.

5. Procédé selon la revendication 1, dans lequel ledit sel de métal alcalino-terreux est le 2,5-dicétogluconate de calcium.

6. Procédé selon la revendication 1, dans lequel ledit co-révélateur est choisi dans le groupe constitué du méthylaminophénol, de la 1-phényl-3-pyrazolidone et des para-phénylènediamines.

7. Produit pour usage photographique contenant une quantité efficace d'une substance révélatrice choisie dans le groupe constitué des sels de métaux alcalins, sels de métaux alcalino-terreux, sels d'amine de l'acide cétogluconique; des sels de métaux alcalins, sels de métaux alcalino-terreux et sels d'amine des stéréoisomères de celui-ci; des esters alkyliques en C₁-C₄ de l'acide cétogluconique, et des esters alkyliques en C₁-C₄ des stéréoisomères de l'acide cétogluconique, et de (b) un co-révélateur dans ledit support photographique.

8. Produit selon la revendication 7, où ledit co-révélateur est choisi dans le groupe constitué du méthylaminophénol, de la 1-phényl-3-pyrazolidone et des para-phénylènediamines.

9. Procédé pour le développement d'une image photographique sur un support photographique comprenant la réduction de l'argent photosensibilisé sur ledit support avec une quantité efficace de 2-cétogluconate de méthyle.

10. Produit pour usage photographique contenant une quantité efficace de 2-cétogluconate de méthyle comme substance révélatrice.

## Revendications (Revendications pour l'(les) Etat(s) contractant(s) suivant(s): BE, DE, FR, GB, IT, NL)

1. Procédé pour le développement d'une image photographique sur un support photographique comprenant la réduction de l'argent photosensibilisé sur ledit support avec une quantité efficace de (a) du 2,5-dicétogluconate de calcium et de (b) un co-révélateur pour ledit support photographique.

2. Procédé selon la revendication 1, dans lequel ledit co-révélateur est choisi dans le groupe constitué du méthylaminophénol, de la 1-phényl-3-pyrazolidone et des para-phénylènediamines.

3. Produit à usage photographique contenant une quantité efficace de 2,5-dicétogluconate de calcium et d'un co-révélateur dans ledit support photographique.

4. Produit à usage photographique selon la revendication 3, où ledit co-révélateur est choisi dans le groupe constitué du méthylaminophénol, de la 1-phényl-3-pyrazolidone et des para-phénylènediamines.
